

## UNITED STATES PATENT OFFICE.

JOSEPH BRINCIL, OF READING, PENNSYLVANIA.

## BEARING AND METHOD OF MAKING IT.

No Drawing.

Application filed September 21, 1926. Serial No. 136,894.

This invention relates to bearings and their manufacture, particularly to bearings of the self-lubricating type.

There is at present on the market, and sold under various trade names, a self-lubricating bearing material in the form of spongy bronze having approximately 40 per cent by volume of graphite mechanically mixed with it and uniformly distributed throughout its mass.

- 10 This material is capable of absorbing about 20 per cent by volume of oil and on the whole forms a very satisfactory bearing. It is, however, expensive to manufacture and difficult to work. The process of making it comprises
- 15 mixing powdered bronze, powdered graphite and a binder and compressing the whole under hydraulic pressure. The resulting product cannot readily be machined and is therefore commonly ground or molded to shape.
- 20 For this reason it can be made into flanged or split bushings only with difficulty and with great waste of material, so that its use is practically limited to very simple shapes. It is, moreover, weak and easily deformed.

- 25 It is the object of the present invention to provide an inexpensive method of making a bearing having substantially the advantages of this costly bronze sponge without its disadvantages. I do this by forming on a strip of bearing metal a surfacing similar to the spongy bronze-graphite described above, which strip can then be readily fashioned into bearings of any desired shape, thus making available the excellent lubricating qualities of the bronze sponge at relatively little expense. I form this spongy or porous surfacing on the bearing metal by first subjecting a strip of that metal to the abrading action of a blast of granular abrasive, coating the abraded surface with a binder and then applying a composition comprising graphite and a binder and preferably including a powdered metal, such as bronze. After drying, the whole is compressed to force the graphite into the interstices of the abraded surface and thus incorporate it with the base metal. The resultant product is a metal strip having an absorbent lubricating face capable of absorbing a small quantity of oil and closely resembling bronze sponge in its bearing properties.

As one specific method of carrying out my

invention I proceed as follows. A roll of metal strip, preferably bronze, about 12 inches wide and 40 or 50 feet long, is unwound from 55 one roll and onto a second receiving roll, passing horizontally through a housing in which its upper face is abraded by means of a blast of granular abrasive directed against it by an operator standing outside the housing. Abrading equipment of this nature is old and of itself forms no part of the present invention so that I have not illustrated it. Any standard abrasive can be used, such as natural or artificial minerals or metal 60 abrasives, such as chilled iron. For the purpose of the present invention, I much prefer the latter because the use of mineral abrasives necessitates the careful cleaning of the treated strip to remove all traces of mineral particles which would be detrimental in a bearing surface. The air pressure used amounts to from 60 to 90 pounds per square inch and the strip is moved through the housing at about 10 feet per minute. This treatment 70 produces on the strip a rough granular surface extending for a depth of about .01 to .015 inch, the physical character of which is unique and is excellently adapted to hold a layer of applied lubricant.

The abraded strip of bearing metal is then cut into units of the desired size which are coated with a thin coating of shellac, or other suitable binder, and upon this is applied a layer of finely divided graphite and a binder. 80 For best results, I prefer to incorporate granular bronze with the graphite in the proportion of about 6 parts of bronze to 4 parts of graphite. The surfaced metal is dried and then subjected to pressure. This may be done 85 by a separate pressing operation, or the pressure may be applied when the ultimate shapes are drawn from the treated metal in accordance with the process described and claimed in my Patent No. 1,583,913. The surfaced 90 material either before or after the final shaping is preferably immersed in hot oil of which an appreciable quantity is absorbed. This improves the lubricating properties of the bearing without interfering with the action of 95 the graphite.

The product of this process has a surface layer which is quite similar in its lubricating properties to the bronze sponge described

above. The strip can, however, be readily shaped to form bearings of any desired configuration and either wound into cylindrical shape to form split bushings, or drawn to shape to form non-split, unitary bushings. Bushings having flanges can also be readily made. It is thus possible to make bearings having all of the advantages of bearings made of bronze sponge but with none of their disadvantages, and much less expensively.

I am aware of Patent No. 1,129,304 granted on the invention of Harry C. Loudenbeck in which is described a method of making a bearing surface by etching a piece of bearing metal and rubbing graphite over the etched surface. The physical condition of the abraded surface made in accordance with my invention is essentially different from the etched surface made by the Loudenbeck method. With an etched surface, it would be impossible to produce the porous, adherent, lubricating surface of my bearing metal.

I claim:

1. The method of making a self-lubricating bearing which comprises abrading the surface of a strip of bearing metal, applying a coating of a binder thereon, applying a lubricating composition comprising a mixture of graphite and powdered bronze to the coated face of the metal, permitting the whole to dry and subjecting it to pressure to unite the graphite and bronze with the abraded surface.

2. The method of making a self-lubricating bearing which comprises abrading the surface of a strip of bearing metal, applying a coating of a binder thereon, applying a lubricating composition comprising a mixture of graphite and powdered bronze to the coated face of the metal, permitting the whole to dry, subjecting it to pressure to unite the graphite and bronze with the abraded surface and impregnating the applied surfacing with oil.

3. The method of making a self-lubricating bearing which comprises abrading the surface of a strip of bearing metal by directing a blast of granular abrasive against it, applying a coating of a binder to the abraded surface, then applying thereto a lubricating composition comprising a mixture of graphite and powdered bronze, permitting the applied surface to dry and then subjecting it to pressure to unite the graphite and bronze with the abraded surface.

4. The method of making a self-lubricating bearing which comprises abrading the surface of a strip of bearing metal by directing a blast of granular abrasive against it, applying a coating of a binder to the abraded surface, then applying thereto a lubricating composition comprising a mixture of graphite and powdered bronze, permitting the applied surface to dry and impregnating the surfaced product with oil.

5. The method of making a self-lubricating bearing which comprises abrading the surface of a strip of bearing metal by directing a blast of granular abrasive against it, applying a coating of a binder to the abraded surface, then applying thereto a lubricating composition comprising a mixture of graphite and powdered bronze, permitting the applied surface to dry, and drawing the metal into cylindrical form.

6. The method of making a self-lubricating bearing which comprises abrading the surface of a base metal, applying thereto graphite, a powdered bearing metal and a binder, and uniting the graphite and powdered metal to the abraded base by means of pressure.

7. The method of making a self-lubricating bearing which comprises abrading the surface of a base metal, applying thereto graphite, a powdered bearing metal and a binder, uniting the graphite and powdered metal to the abraded base by means of pressure, and impregnating the surface with oil.

8. The method of making a self-lubricating bearing which comprises abrading the surface of a strip of base metal, applying thereto graphite, a powdered bearing metal and a binder, uniting the graphite and powdered metal to the abraded base by means of pressure, and shaping the strip into cylindrical form.

9. The method of making a self-lubricating bearing which comprises abrading the surface of a base metal, applying a coating of a binder thereon, applying a lubricating composition comprising a mixture of graphite and powdered bronze to the coated face of the metal and subjecting it to pressure to unite the graphite and bronze with the abraded surface.

10. The method of making a self-lubricating bearing which comprises abrading the surface of a base metal, applying thereto a powdered bearing metal and a binder, and uniting the powdered metal to the abraded base by means of pressure.

11. A self-lubricating bearing composition comprising a metal base having an abraded surface and a layer of graphite and powdered bearing metal in the cold state united to said abraded surface and capable of absorbing a lubricating oil.

12. A self-lubricating bearing composition comprising a metal base having an abraded surface and a spongy layer of graphite and powdered bearing metal in the cold state united to said abraded surface, and impregnated with a lubricating oil.

13. A self-lubricating bearing in cylindrical form comprising a metal base having an abraded surface and a spongy layer of graphite and powdered bearing metal in the cold state united to said abraded surface.

14. A self-lubricating bearing in cylindrical form comprising a metal base having an abraded face and a spongy bearing surface.

united to said abraded face comprising powdered bearing metal in the cold state.

15. A self-lubricating bearing comprising a metal base having an abraded surface and a layer of graphite and powdered bronze in the cold state united to said abraded surface, and capable of absorbing oil.

16. A self-lubricating bearing comprising a base of bronze having an abraded surface, and a spongy layer of graphite and powdered bronze in the cold state united to said abraded surface.

In testimony whereof I affix my signature.

JOSEPH BRINCIL.